

H. H. ASHDOWN.  
CASTING STEEL INGOTS.  
APPLICATION FILED JUNE 18, 1917.

1,251,951.

Patented Jan. 1, 1918.



Inventor:  
Herbert Henry Ashdown,  
By his attorneys  
*Baldwin & Wright.*

# UNITED STATES PATENT OFFICE.

HERBERT HENRY ASHDOWN, OF NEWCASTLE-UPON-TYNE, ENGLAND, ASSIGNOR TO  
SIR W. G. ARMSTRONG, WHITWORTH AND COMPANY, LIMITED, OF NEWCASTLE-  
UPON-TYNE, ENGLAND.

## CASTING STEEL INGOTS.

1,251,951.

Specification of Letters Patent.

Patented Jan. 1, 1918.

Application filed June 18, 1917. Serial No. 175,487.

*To all whom it may concern:*

Be it known that I, HERBERT HENRY ASHDOWN, a subject of the King of Great Britain, residing at Elswick Works, Newcastle-upon-Tyne, England, have invented a new and useful Improvement in Casting Steel Ingots, of which the following is a specification.

This invention relates to the casting of ingots and has for its object the prevention of segregation of the non-metallic material in the greater part of the body of the ingot and of the formation of corner cracks.

According to this invention the sides of the ingot are first cooled until the metal has solidified preferably to a considerable thickness, and the ingot is then cooled from its base upward in order to effect the solidification of the still liquid central portion from the base upward. By this process segregation is confined to the top of the ingot.

The casting may take place in any form of mold, but the drawing which is annexed to this specification and which is an elevation partly in section, illustrates a mold suitable for the purpose.

A is a mold having a bottom plate B and in the mold and plate are pipes D for the circulation of the cooling medium, the supply to the various pipes being controlled by a series of cocks E. The cooling medium is discharged from the pipes D by pipes F.

By opening the lowest cock E the bottom plate alone is cooled, and similarly any section of the mold may be cooled as desired.

In casting the ingot the metal is fed through a feeding head C of usual construction, and in the course of usual working the cocks E are opened in succession upward as the liquid metal reaches the part of the mold cooled by each section of pipes.

The effect of this is to promote a much quicker solidification of the metal in proximity to the cooled walls of the ingot mold for the entire length of the ingot, causing the segregates to be forced to the center of the ingot.

In some cases, especially when very large ingots are being cast, the operation takes a

considerable time and the upper portion of the mold becomes hot before the level of the metal gets up to it, and it may be desirable to cool this portion of the mold early in the operation. Similarly the cooling effect of the bottom plate and the lowest portion of the mold may be sufficient to solidify the bottom of the ingot without the assistance of the cooling medium, so that it is not always necessary to open the lowest cocks at the commencement of the operation.

Finally after the pouring of the metal is finished the cooling effect of the lowest cooling coil in the wall of the mold and the coil in the bottom plate is increased so that the central portion of the metal which is still liquid is cooled from its bottom end upward forcing the segregates into the last portion remaining liquid near the feeding head.

What I claim is:—

1. The process of casting ingots, which consists in pouring the ingot, subjecting the same to an advancing cooling action corresponding to the advancing formation of said ingot, and after completion, again submitting the ingot to a further cooling action.

2. The process of casting ingots, which consists in pouring the ingots, and during the pouring action subjecting the successive accretions to a correspondingly advancing cooling action.

3. The process of casting ingots, which consists in pouring the ingot, during the pouring action subjecting the successive accretions to a correspondingly advancing cooling action, and after the completion of the ingot again subjecting said ingot to an additional cooling action extending from one end toward the other.

4. The process of casting ingots, which consists in pouring the metal into a mold, subjecting the mold to a cooling action during the pouring operation, and after the completion of the pouring action again subjecting the mold to a cooling action that advances from the bottom toward the top.

5. The process of casting ingots, which consists in pouring the metal into a mold,

subjecting the mold to a cooling action during the pouring operation, said cooling action being advanced along the mold as the filling takes place, and afterward again subjecting the mold to a cooling action that advances from the bottom toward the top.

5 In testimony that I claim the foregoing

as my invention I have signed my name this  
25th day of May 1917.

HERBERT HENRY ASHDOWN.

Witnesses:

H. NIXON,

A. MITCHINSON.